

# UNITED STATES PATENT OFFICE.

SILAS R. DIVINE, OF LOCH SHELDRAKE, NEW YORK, ASSIGNOR TO THE  
REND ROCK POWDER COMPANY, OF NEW JERSEY.

## EXPLOSIVE COMPOUND.

SPECIFICATION forming part of Letters Patent No. 289,757, dated December 4, 1883.

Application filed July 23, 1883. (No specimens.)

*To all whom it may concern:*

Be it known that I, SILAS R. DIVINE, of Loch Sheldrake, Sullivan county, State of New York, and a citizen of the United States, 5 have invented an Improvement in Explosive Compounds, of which the following is a full, clear, and exact specification.

The object of my invention is to "sensitize" or impart increased susceptibility to explosion 10 to an explosive compound for use, chiefly, in blasting, composed of chlorate of potash and nitro-benzole, so that the said compound may be readily exploded under various conditions of confinement, as in loose or "rotten" rock or shale, or in earth, or in the open air.

My invention consists in an explosive compound composed of chlorate of potash and nitro-benzole substantially in the proportions of from 20 about three to four and one-sixth parts of the former to one part of the latter, (as described by me in Letters Patent No. 243,432, dated June 28, 1881,) with the wet or moist mass of which said ingredients is united sulphur in a finely-powdered state in the proportions hereinafter stated.

As is stated in said Letters Patent above referred to, either perchlorate or permanganate of potash may be employed in place of chlorate of potash in the compound, and, in like manner, other liquid nitro compounds 30 may be substituted for the nitro-benzole, and the theoretical proportions in which these said ingredients combine most effectively to form 35 an explosive may be varied somewhat and still

an effective explosive be constituted; and, furthermore, the chlorate of potash being in a crushed or powdered state and used as the solid ingredient, and the nitro-benzole being used as the liquid ingredient of the compound, these two ingredients may be readily combined by simply allowing the said solid to absorb the liquid.

The proportion in which it is desirable to use the sulphur is from about one to three 45 per cent. thereof relatively to the mass of the combined two other ingredients named; but these proportions may be varied without departing from the essential feature of this invention. The sulphur is united with the wet or moist mass of the combined chlorate of potash and nitro-benzole, and this may be accomplished by mixing the sulphur with said mass by hand in a suitable vessel.

The danger of accidental explosion attendant upon mixing sulphur with chlorate of potash in a dry state is thus avoided.

What I claim as my invention, and desire to secure by Letters Patent, is—

The explosive compound herein described, composed of chlorate of potash and nitro-benzole, substantially in the proportions named, with the wet or moist mass of which said combined ingredients is united sulphur in substantially the relative proportions, and as and 65 for the purpose set forth.

SILAS R. DIVINE.

Witnesses:

A. G. N. VERMILYA,  
A. S. FITCH.